

Patented Feb. 6, 1923.

1,444,723

# UNITED STATES PATENT OFFICE.

LINDON WALLACE BATES, OF MOUNT LEBANON, NEW YORK.

## METHOD OF TREATING STABLE MOBILE FUELS.

No Drawing.

Application filed February 6, 1920. Serial No. 356,689.

To all whom it may concern:

Be it known that I, LINDON W. BATES, a citizen of the United States, and resident of Mount Lebanon, in the county of Columbia 5 and State of New York, have invented certain new and useful Improvements in Methods of Treating Stable Mobile Fuels, of which the following is a specification.

This invention pertains to a process in the 10 fuel art. More specifically it pertains to the transformation of the stable mobile fuel described in my copending application, Serial No. 315,497, filed on August 5, 1919, Patent No. 1,390,228, September 6, 1921 directed 15 toward a "Fuel and method of producing same." The said fuel called "Colloidal fuel" consists of particles of solid carbonaceous substance and liquid hydrocarbon stabilized by the use of certain substances 20 and by the mechanical or heat treatment or both appropriate for properly commingling the components. Among the stabilizing substances may be mentioned lime-rosin grease and coal distillates or equivalent stabilizing 25 or stabilizing and peptizing materials. The particles in the fuel are found in three states of dispersion, the molecular, colloidal and suspension. This is due to the fact that the carbonaceous substance is reduced by pul- 30 verization or otherwise so that about eighty-five per cent passes a two hundred mesh screen. In a batch of coal, for example, so pulverized most of the particles are of suspension size, while comparatively smaller 35 quantities are reduced to colloidal dimensions or to molecules. Up to 40% by weight of particles may be carried in a liquid fuel and 75% in a paste. This tri-state fuel is excellent for burning and for gas making 40 purposes in particular, and may also be used in Diesel engines and semi-Diesel engines when the scavenging system is adjusted thereto. Liquids or pastes may form gels.

On the other hand a composite fuel which 45 contained only colloidal and molecular particles could be used in internal combustion engines without change in the scavenging system from its oil adjustment. Colloids of coal in oil for use in internal combustion engines are known, but only small amounts of carbonaceous substance have been so reduced and to accomplish the result it has been necessary heretofore to reduce material of suspension size to colloidal size by disk grinding or hammering with lengthy trituration 50 at high speed or high pressure, a method

unsuited to industrial needs. It has been found, however, that a fuel suitable for internal combustion engines without apparatus changes may be obtained from the tri-state fuel described in my copending application. This invention proposes to treat the said fuel in such a fashion as to produce therefrom two distinct varieties. The one variety is a colloid-like liquid combustible 60 of moderate viscosity containing particles of carbonaceous substance many of which are in the colloid and molecular state and some of which are in the suspension state. The other is a paste in which the carbonaceous 65 particles are mostly of suspension size. To produce these two varieties it is necessary to add one or more steps to the colloidalizing process described in my copending application. The result may be accomplished by 70 separating all or some of the suspension particles from the colloidal fuel.

Suspension particles may be removed in a number of ways from the tri-state fuel as produced. For example, the fuel may be 80 centrifuged, which separates out a considerable portion of the larger particles. Or again the equilibrium of stability of the fuel may be modified by reducing its viscosity very materially, as by prolonged and extreme heat or as by adding benzol, alcohol or some other suitable liquid or substance, and then allowing the suspension particles to settle out. Another way to separate the components is to force the fuel through 85 cheese cloth, linen, filter paper or porcelain. Such treatment retains on the filter or screen many of the larger particles, and in the case of porcelain filters only the colloidal and molecular particles pass with the oil.

The liquid fuel remaining after the removal of centrifuged particles is practically colloidal coal in oil, since most of the larger particles have been removed. The same is true of the tri-state fuel whose stability has 90 been terminated as regards the larger particles when these have been removed upon settling. If a fine filter is used a true colloid may be obtained. A combination of these methods may be employed. In practice it is 100 not necessary to remove all the suspension particles, as internal combustion engines can readily use without changes a liquid fuel which is not filled with a multiplicity of particles of suspension size. The further 110 treatment herein described may stop short therefore of a transformation of the tri-

state fuel into one or more mono or bi-state fuels.

It is entirely possible also to take the internal combustion engine fuel produced from 5 colloidal fuel and to recolloidalize it, adding further carbonaceous particles. Particles of suspension size in the new lot added may also be removed, leaving a produce richer in colloidal and molecular particles.

10 The removed larger particles carry with them a certain number of the smaller particles and associated oil or liquid, and form a fuel paste which is of economic value. The paste is not necessarily wholly in the suspension state, inasmuch as particles within colloidal dimensions are still found in it. This 15 paste may be used as such or may be treated with further oil or liquid to form a more fluid fuel similar to the original colloidal 20 fuel but containing fewer colloidal particles.

Or again the paste residue after the removal of the lighter fuel from the separated particles may be briquetted or otherwise 25 dealt with as desired. To make a briquette or a road compound it may be necessary to add hardening substances.

The process herein described results in the production of two varieties of colloidal 30 fuel or really sub-varieties. From the original fuel containing particles in three states of dispersion, two varieties have been derived, the one containing most of the colloidal and molecular particles of that fuel, 35 and the other containing most of the suspension particles. Each of these varieties of the same basic fuel may be still further treated in view of the different classes of uses for which it is adapted.

40 It may be advantageous to add internal combustion engine fuel or like liquid hydrocarbon to the liquid variety. Thus alcohol or gasoline may be used therewith. The treatment does not adversely affect the stability of the two varieties, each of which 45 will be stable. In fact, the stability of the

liquid variety is enhanced. The two varieties may each serve a useful purpose and may undergo further transformations before use.

50 Since a perfect separation of the suspension particles is not to be anticipated each of the products resembles fuel products covered in my said copending application, but the method of producing the new varieties differs 55 in the present case from the original colloid-alizing process in view of the additional steps. As these products are all simply further examples of the fuel covered by my copending application, I do not claim herein 60 the said products but I do claim the method involving the additional process steps which are employed to produce them.

Having thus stated the nature of my invention what I claim is:

65 1. That method of producing a stable liquid fuel which consists in pulverizing solid carbonaceous substance so that approximately 85% would pass a 200 mesh screen, commingling the same with liquid hydrocarbon and stabilizing substance, and removing suspension-sized particles.

70 2. That method of producing a stable liquid fuel which consists in pulverizing solid carbonaceous substance so that approximately 85% would pass a 200 mesh screen, 75 commingling the same with liquid hydrocarbon and stabilizing substance, removing suspension-sized particles; and adding further liquid hydrocarbon to the remaining liquid. 80

3. That method of producing a stable liquid fuel which consists in pulverizing solid carbonaceous substance so that approximately 85% would pass a 200 mesh screen, 85 commingling the same with liquid hydrocarbon and a small amount of lime-rosin soap or equivalent stabilizing substance, and removing suspension sized particles.

Signed at New York city, in the county of New York and State of New York, this 4th 90 day of February, A. D. 1920.

LINDON WALLACE BATES.